

Aug. 3, 1954

O. F. DAVIS ET AL

2,685,121

METHOD AND APPARATUS FOR MANUFACTURE OF METAL FILMS

Filed May 7, 1949

FIG. 1.



FIG. 2.



INVENTORS  
OLIVER F. DAVIS,  
HANS G. BELITZ,  
by

Toulmin & Toulmin  
ATTORNEYS

## UNITED STATES PATENT OFFICE

2,685,121

## METHOD AND APPARATUS FOR MANUFACTURE OF METAL FILMS

Oliver F. Davis, Troy, and Hans G. Belitz, Dayton, Ohio, assignors to The Commonwealth Engineering Company of Ohio, Dayton, Ohio, a corporation of Ohio

Application May 7, 1949, Serial No. 91,924

9 Claims. (Cl. 29—17)

1

This invention relates to metal foil. More particularly, it relates to a continuous method of producing metal foil or film. Still more particularly it relates to film formation by continuous deposition of metal from the vapor state.

In the past metal foils have been produced by preparing billets of malleable metals or malleable alloys and passing the billets between rollers, which reduced the thickness of the billet by stages.

In the final stages the metal is passed between very accurately machined rolls, and simultaneously therewith the thin metal sheet issuing from between the rolls is drawn by careful application of tensioning stress. The thin drawn metal sheet is then wound on reels for storage and shipping.

This process is costly and requires large and expensive equipment. In the final stages the maintenance of tension is a delicately balanced operation, which requires constant attention to avoid overstressing the metal and breaking the foil.

Further, the maintenance of accurately machined close clearance rolls, such as are required for the final stages of foil preparation, is a constant expense.

It is an object of the present invention to overcome the disadvantages and the necessity for costly equipment enumerated above.

A further object of the present invention is to produce foils or films by deposition of metal.

A still further object of the invention is to produce foils or films without the necessity for expensive roller equipment.

Another object of the present invention is to produce thin foils or films of any metal which can be deposited from the vapor state.

A further object of the invention is to provide foils of durable structure and excellent fatigue resistance.

Another object of the invention is to provide a process in which a thin film of metal is continuously deposited and the deposited film continuously removed from a revolving base.

A still further object of the invention is to provide apparatus wherein the gaseous medium bearing metal is directed into contact with a rotating heated surface.

In brief, the process consists of impinging a stream of vapor bearing depositable metal upon a continuously rotating cylindrical base or roll. This rotating base is provided with a smooth prepared surface, to which the deposited metal has little adherence.

The non-adhering coating, generally having

2

a thickness of .005 to about .025 inches, is then stripped from the cylindrical base and the foil removed from the plating chamber for cooling and winding on reels.

5 This process is given over to the production of two similar types of foil. One type is produced by depositing upon the base a thin insulating layer of thermoplastic resin which is stripped from the base and remains on the foil.

10 The other type of foil is produced by depositing upon the base a thin insulating coating of material which prevents the deposited metal from adhering tightly to the base, but which can be easily removed by a simple washing operation. These insulating layers are usually between about .000005 to .0005 inches in depth.

Certain of the insulating materials may be used in conjunction with the resins, if desired, but their presence usually necessitates a removal step.

15 Conditioning of the base against adherence of deposited metal may be accomplished by blowing powdered graphite on to the roll or base, or by continuously sizing the roll with a wax or resin which does not soften appreciably at a temperature, for example, of 400° F., the temperature at which many carbonyls and hydrides decompose to deposit their metal component.

20 One simple method of preventing adherence is to cause the drum to rotate in a smoky acetylene flame which deposits carbon soot.

25 Metals which may be deposited as thin films are, for example, nickel, chromium, copper, tungsten, tin, zinc, lead, and the like.

30 One particularly advantageous method of bringing metal as vapors into the plating zone is in the form of readily decomposable gaseous compounds. For example, the metals may be introduced as gaseous metal carbonyls, also nitrosoyl compounds, nitrosyl carbonyls, metal hydrides, metal alkyls, metal halides, and the like.

35 Illustrative compounds of the carbonyl type are nickel, iron, chromium, molybdenum, cobalt, and mixed carbonyls.

40 Illustrative compounds of other groups are the nitrosoyls, such as copper nitrosoyl; nitrosyl carbonyls, for example, cobalt nitrosyl carbonyl; hydrides, such as antimony hydride, tin hydride; metal alkyls, such as tetraethyl lead; metal halides, such as chromyl chloride; and carbonyl halogens, for example, osmium carbonyl bromide, rhuthenium carbonyl chloride, and the like.

45 The plating of foil or film may be carried out under a wide variety of conditions. When undiluted vapors are fed to the plating zone, it is

generally preferable to feed the vapors under a slight positive pressure, i. e. a pressure above atmospheric. When dilute vapors are fed to the plating zone, an even wider range of pressures may be used, running from negative pressures usually expressed in inches of water vacuum to positive pressures usually expressed as pounds per square inch gage.

The manner in which the metal bearing vapors are entrained varies from carbureting metal vapors into an inert gas stream maintained under pressure to spraying liquid into hot gas being sucked through the system by vacuum, which gas vaporizes the liquid droplets whereby the liquid is a vapor in the plating zone.

Each material from which metals may be plated has a temperature at which the metal in vapor form is free to deposit as a metal coating. When plating there is an optimum plating range for a large number of, for example, metal carbonyls, running from about 350° F. to 450° F. Decomposition takes place outside this range, but when seeking uniform deposits, it is desirable to operate within the above range and even within the range of 375° F. to 400° F., if it is desired to plate nickel, molybdenum, cobalt, and the like.

The above mentioned 350° F. to 450° F. temperature range is also useful for decomposition of many of the hydrides. However, since each type of metal and each type of compound alters the plating range, applicants merely offer the above as a range for specific embodiments of the invention and not as a limitation upon the operating range of coating deposition.

The invention will be more fully understood by reference to the drawing:

Figure 1 is a vertical sectional view of apparatus illustrating one embodiment of the invention; and

Figure 2 is a plan view showing the relationship of the vapor conductor hood to the metal plating roll.

The apparatus consists of a chamber 10 which is provided with a jacket 11. Chamber 10 is also provided with a gas outlet 12 which may, if desired, be connected to exhaust means (not shown) such as an exhaust fan or vacuum pump.

Jacket 11 is provided with inlet means 13 and outlet means 14 for introduction and removal of cooling medium from the jacket.

Mounted within the chamber 10 is a cylindrical roll or drum 16 of suitable construction material such as glass. Drum 16 is supported on a shaft 17 suitably journaled in the walls of chamber 10 and driven by a prime mover such as an electric motor stationed outside the chamber through a suitable coupling and speed reduction gear.

Drum 16 is provided internally but adjacent its peripheral area with heating means 20, such as electrical resistance coils, induction coils, and the like, whose electrical circuit is connected to a source of power through a suitable brush arrangement mounted on shaft 17.

Metal bearing gases are introduced into chamber 10 through conduit 21. Conduit 21 is provided at its inner end with a hood like portion 22 adapted to direct inflowing gases into contact with a large area of the surface of the roll.

Tangentially positioned in contact with the exterior of the roll 16 is a doctor blade 23 adjustable by screw 24. This blade serves for stripping coated deposits from the roll.

Metal stripped from the roll by the doctor blade is directed between rollers 25 closing the aper-

ture 26 in the end section 27 of chamber 10. End section 27 is jacketed by a gas chamber 28 which is adapted with inlet means 29 and outlet means 30 for introduction and venting of an inert gas atmosphere.

Metal strip issuing between rollers 25 traverses the chamber 28 and passes between rollers 31 in the opposite wall of the gas chamber 28 to reel winding equipment (not shown).

In the operation of this equipment a layer, for example, of wax is deposited on the drum 16 by the feeder 35. The wax sets during the slow travel of the drum through 90 degrees from the point of application.

The drum is maintained at a temperature of approximately 400° F. In order to start a run a thin layer of copper is passed between the rollers 31 and 25 and is molded to conform to the shape of the roll 16.

A stream of, for example, nickel carbonyl vapors flowing at the rate of 150 cubic feet per hour, diluted with carbon dioxide is brought into contact with the roll 16 through conduit 21.

The carbon dioxide and gaseous decomposition products are exhausted through outlet means 12. When deposition has become appreciable winding of the reel and rotation of roll 16 is initiated.

Due to the adherence of nickel to copper the nickel film is drawn out through lock rollers 25, is cooled in an inert atmosphere while traversing chamber 28, and is passed through the lock rollers 31 to the winding reel.

Chamber 28 is maintained under a slightly higher gas pressure than chamber 10 which action prevents leakage of toxic gases from chamber 10.

While the method and apparatus disclosed and described herein illustrate a preferred form of invention, yet it will be understood that modifications can be made without departing from the spirit of the invention, and that modifications that fall within the scope of the appended claims are intended to be included herein.

We claim:

1. The method of preparing metal foil which comprises, maintaining a cylindrical roll in continuous revolving motion, coating a substantially cleared surface of the roll with an adherence-reducing medium, heating said roll to a temperature in the range of 350° F. to 450° F., impinging a gaseous stream of inert gas and metal carbonyl against said heated revolving roll whereby the carbonyl is decomposed and the metal deposited to produce a thin film on said roll, and continuously stripping the thin film of deposited metal from said roll.

2. The method of preparing metal foil which comprises, maintaining a cylindrical roll in continuous revolving motion, coating a substantially cleared surface of the roll with an adherence-reducing medium, heating said roll to a temperature in the range of 350° F. to 450° F., impinging a gaseous stream of inert gas and a metal carbonyl against said heated revolving roll whereby the carbonyl is decomposed and the metal deposited to produce a thin film on said roll, and continuously stripping the thin film of deposited metal from said roll, said metal carbonyl being selected from the group consisting of nickel carbonyl, iron carbonyl, and cobalt carbonyl.

3. The method of preparing metal foil which comprises, maintaining a cylindrical roll in continuous revolving motion, coating a substantially cleared surface of the roll with an adherence-reducing medium, heating said roll to a tem-

perature in the range of 350° F. to 450° F., impinging a gaseous stream of inert gas and metal hydride against said heated revolving roll whereby the hydride is decomposed and the metal deposited to produce a thin film on said roll, and continuously stripping the thin film of deposited metal from said roll.

4. The method of preparing metal foil which comprises, maintaining a cylindrical roll in continuous revolving motion, coating a substantially cleared surface of the roll with an adherence-reducing medium, heating said roll to a temperature in the range of 350° F. to 450° F., impinging a gaseous stream of inert gas and a metal hydride against said heated revolving roll whereby the hydride is decomposed and the metal deposited to produce a thin film on said roll, and continuously stripping the thin film of deposited metal from said roll, said metal hydride being selected from the group consisting of tin hydride and chromium hydride.

5. The method of preparing metal foil which comprises, maintaining a cylindrical roll in continuous revolving motion, coating a substantially cleared surface of the roll with Carnauba wax, heating said roll to a temperature of approximately 390° F., impinging a gaseous stream of carbon dioxide and nickel carbonyl against said heated revolving roll whereby the carbonyl is decomposed and the nickel is deposited on said roll in film form to a depth of approximately .025 inch, maintaining a pressure in the coating area of approximately 3 inches of water vacuum, and continuously stripping the nickel film from said roll.

6. Apparatus for the preparation of metal foils comprising a chamber, a cylindrical roll mounted within said chamber, means for rotating said roll, means for heating said roll, means for introducing heat-decomposable metal bearing vapors into contact with said roll, outlet means for removing vapors from said chamber, and cutting means in contact with said roll for stripping deposited metal film from said roll.

7. Apparatus for the preparation of metal foils comprising a chamber, a jacket associated with said chamber, inlet and outlet means for circulation of cooling medium in said jacket, a cylindrical roll mounted within said chamber, means for rotating said roll, heating means within said roll, conduit means for introducing heat-decomposable metal compound vapors into contact with the outer surface of said roll, conduit means for removal of gases from said chamber, and cutting means tangential to the surface of said roll and in contact therewith for stripping deposited metal from said roll.

8. Apparatus for the preparation of metal foils comprising a primary chamber, a jacket associated with said chamber, a secondary chamber, inlet and outlet means for circulating gaseous medium, gas tight roller locks between the primary and secondary chamber for passage of foil therebetween, and locking rollers for removal of foil from secondary chamber to reeling apparatus.

9. In a method of preparing metal foil comprising the steps of depositing a thin metal coating on a rotating cylinder, the improvement which consists in depositing the metal forming the foil as a heat-decomposable gaseous metal compound, and wherein said cylinder is heated to a temperature sufficient to cause said gaseous metal compound to be decomposed and the metal component thereof deposited as a thin layer on the surface of said cylinder.

References Cited in the file of this patent

UNITED STATES PATENTS

| Number    | Name     | Date          |
|-----------|----------|---------------|
| 2,344,138 | Drummond | Mar. 14, 1944 |

FOREIGN PATENTS

| Number  | Country       | Date          |
|---------|---------------|---------------|
| 14,845  | Great Britain | June 21, 1907 |
| 17,115  | Great Britain | July 19, 1910 |
| 39,453  | Denmark       | Oct. 27, 1928 |
| 454,919 | Great Britain | Oct. 5, 1936  |